

# UNITED STATES PATENT OFFICE.

EDWARD JOHN BEVAN, OF LONDON, ENGLAND.

## ABSORBENT FOR CARBON DIOXID IN BREATHING APPARATUS FOR USE IN MINE-RESCUE WORK OR LIKE PURPOSES.

1,223,244.

Specification of Letters Patent. Patented Apr. 17, 1917.

No Drawing.

Application filed November 17, 1915. Serial No. 61,993.

To all whom it may concern:

Be it known that I, EDWARD JOHN BEVAN, a subject of the King of Great Britain, residing in London, England, have invented a certain new and useful Improved Absorbent for Carbon Dioxid in Breathing Apparatus for Use in Mine-Rescue Work or like Purposes, of which the following is a specification.

10 In breathing apparatus, such as is used in mine rescue work and for like purposes, the carbon dioxid exhaled is absorbed by caustic alkali. The forms in which the alkali, generally caustic soda, has commonly been used are not satisfactory, partly because they become very hot during the absorption and partly because they deliquesce and then offer resistance to respiration. The first objection is mainly due to the high heat of hydration of the alkali and could be overcome by the use of a previously hydrated alkali, such as a strong solution; the latter, however, is as objectionable as the deliquesced alkali referred to above.

25 By the present invention the absorption chamber of the apparatus is charged with a material made by grinding cellulose preferably wood pulp, with a strong solution of caustic alkali, preferably soda. This material is itself known as an intermediate product in the manufacture of viscose, and one method of preparing it consists in incorporating by means of an edge runner 3 lbs. of caustic soda liquor containing 1 lb. of caustic 30 soda with 2 lbs. of ground wood pulp; the material thus prepared resembles bread crumbs, except in color. It was not to be foreseen that this material would have special advantages as an absorbent in the kind 35 of apparatus in question. These advantages

are that, since it contains the alkali in a more or less completely hydrated condition, it does not become hot during the absorption; that it exposes, per unit weight, a very large surface coated with caustic soda, so 45 that a given bulk of it is a better absorbent and of much less weight than the same bulk of caustic soda in lumps or sticks; that it does not deliquesce; that it is easy to handle. In the last three respects, it also surpasses 50 any mineral material, such as pumice, saturated with hydrated alkali.

Having thus described the said invention and the best means I know of carrying the same into practical effect, I claim:—

55 1. A material for absorbing carbon dioxid in breathing apparatus for mine rescue work and similar purposes, which material consists of cellulose saturated with hydrated caustic alkali.

60 2. A material for absorbing carbon dioxid in breathing apparatus for mine rescue work and similar purposes, which material has the form of bread crumbs and consists of cellulose saturated with hydrated caustic 65 alkali.

65 3. A material for absorbing carbon dioxid in breathing apparatus for mine rescue work and similar purposes, which material has the form of bread crumbs and consists of ground 70 wood pulp saturated with 150 per cent. of its weight of caustic soda solution of 33 per cent. strength.

75 In testimony whereof I have signed my name to this specification in the presence of two subscribing witnesses.

EDWARD JOHN BEVAN.

Witnesses:

JOSEPH MILLARD,  
W. I. S. KERKAN.

Copies of this patent may be obtained for five cents each, by addressing the "Commissioner of Patents, Washington, D. C."